

No. 881,029.

PATENTED MAR. 3, 1908.

A. SANG.

METHOD OF COATING METALS.

APPLICATION FILED APR. 13, 1907.



WITNESSES

R.A. Alderson  
W.W. Schwartz

INVENTOR

Alfred Sang  
by Baxendell & Byrnes  
his attorneys

# UNITED STATES PATENT OFFICE.

ALFRED SANG, OF SEWICKLEY, PENNSYLVANIA.

## METHOD OF COATING METALS.

No. 881,029.

Specification of Letters Patent. Patented March 3, 1908.

Application April 13, 1907. Serial No. 367,916.

*To all whom it may concern:*

Be it known that I, ALFRED SANG, of Sewickley, Allegheny county, Pennsylvania, have invented a new and useful Method of 5 Coating Metals, of which the following is a full, clear, and exact description, reference being had to the accompanying drawing, forming part of this specification, in which the figure is a diagrammatic sectional side 10 elevation showing one form of apparatus for carrying out my invention.

This invention relates to a method of depositing zinc or other protective metal coatings upon metal objects or articles, to protect 15 them from oxidation or corrosion or for other purposes.

In carrying out my invention, the articles to be coated are preferably first cleaned by any of the well-known methods, such as pickling, sand-blasting, &c., and are then placed 20 in a receptacle which is preferably of metal, though other materials may be used, which is then covered and sealed. This coating box or receptacle is connected by a pipe or 25 conduit with a retort or pot containing the dust of the coating metal. In the case of zinc, this dust will preferably be the ordinary commercial zinc dust which contains some 30 oxid of zinc. If the metal dust does not contain oxid, such oxid should be added to it. I also preferably employ a reducing or fixing 35 agent, such as cyanid of potassium, asphaltum, coal oil, or other reducing agent or agents which may be placed in the retort, in the coating box, or applied as a coating on 40 the articles in the box. The proportion of the reducing agent may be varied widely without materially affecting the result. The pot or retort containing the zinc dust is then 45 heated to a point below the melting point, but sufficient to vaporize this zinc dust. The temperature is preferably from two hundred to five hundred degrees centigrade, though this may be varied within certain 50 limits, depending upon the vaporization point of the particular metal dust employed. The coating receptacle is also preferably heated in order to prevent the deposition of the coating metal upon its inner surface, and 55 this temperature may be varied widely, though I prefer to heat the box from about two hundred to three hundred degrees centigrade.

In the form of apparatus shown in the

drawings, 2 is the retort containing the metal 55 dust and reducing agent, 3 the coating box containing the metal articles 4, and 5 is the pipe connecting the boxes in which I preferably provide a central valve 5<sup>a</sup>. I have shown the retort as mounted in a setting connected to an external combustion chamber 6, the gases passing from the setting through a flue 7 containing the coating receptacle on their way to the stack flue.

8 and 9 represent the removable covers of 65 the retort and coating box respectively, these preferably having flanges seating in grooves containing asbestos gaskets, or similar packing material.

When the dust in the retort is heated to the 70 vaporizing point, the vapor from the dust passes into the coating receptacle, reacts with the reducing agent and deposits the coating metal upon the articles. This coating is of a tough, strongly adherent character, 75 and under most conditions is of a fine granular nature and bright, or else crystalline in character. It is substantially amalgamated or alloyed with the surface portion of the article itself.

The depth or thickness of the coating or deposit may be varied, according to the length of time which the operation is continued, the temperature employed, &c. Pyrometers 10 and 11 are preferably employed for 85 the pot or retort, and also the coating receptacle, so that the heat may be kept within desirable limits.

Instead of supplying the reducing agent in the retort or pot with the metal dust, it may 90 be applied to the articles in the coating receptacle. In such case I have found that where asphaltum is used as a reducing agent forming a coating on the article, the zinc or other metallic deposit will be formed under 95 the asphaltum. This is of especial advantage in structural steel, since the structural shape will not only be provided with the protective metallic coating, but this coating in turn covered by the asphaltum, without any 100 further operation. Articles provided with a covering of paint or non-metallic materials may thus be provided with a metallic coating under the non-metallic covering, using the reducing agent in either receptacle, or as the 105 non-metallic coating itself.

I have found that where either asphaltum, bitumen, heavy oil or similar material is used

with the metal dust, a double coating is given, the inner coating being metallic and the outer one non-metallic.

The advantages of my invention will be apparent to those skilled in the art. The articles do not need to be brought into contact with the metal dust, and large and heavy articles may be treated cheaply and easily. The coating is of the highly desirable tough adherent character. The process may be carried out by placing the articles in the same pot or receptacle with the dust, and without contact therewith; metal dust other than zinc may be employed; and many other changes may be made without departing from my invention.

I claim:—

1. The process of depositing coating metal upon a metallic surface, consisting in vaporizing the dust of the coating metal, and subjecting the metal surface to be coated to the action of said vapor while out of contact with the dust; substantially as described.
2. The method of coating metal surfaces, consisting in heating and vaporizing the dust of the coating metal, treating the vapor with a reducing agent, and depositing the vapor upon the surface to be coated while said surface is out of contact with the metal dust; substantially as described.
3. The method of coating metal surfaces, consisting in vaporizing the dust of the coating metal in the presence of a reducing agent, heating the surface to be coated, and sub-

jecting it to the action of said vapor while out of contact with the dust; substantially as described.

4. The process of depositing coating metal upon a metallic surface, consisting in vaporizing the dust of the coating metal by applying heat of a temperature below the vaporizing temperature of the metal itself, and subjecting the metal surface to be coated to the action of said vapor, while out of contact with the dust; substantially as described. 45

5. The process of simultaneously coating a metallic surface with metallic and non-metallic layers, consisting in vaporizing the dust of the coating metal, and subjecting the metal surface to be coated to the action of 50 said vapor in the presence of the vapor of a non-metallic material while out of contact with the dust; substantially as described.

6. The process of double coating a metallic surface, consisting in vaporizing the dust of the coating metal; and subjecting the metal surface to be coated to the action of said vapor while out of contact with the dust and in the presence of the vapor of a non-metallic material, which acts as a reducing agent for 60 the metallic vapor and gives an additional coating; substantially as described.

In testimony whereof, I have hereunto set my hand.

ALFRED SANG.

Witnesses:

JOHN MILLER,  
H. M. CORWIN.